

A. H. BEALE.  
METHOD OF ROLLING METAL SHEETS.  
APPLICATION FILED MAY 11, 1908.

926,233.

Patented June 29, 1909.

*Fig. 1.*



*Fig. 2.*



WITNESSES

R A Balderson  
G B Bluming

INVENTOR

Adrian H. Beale  
By Balances, Bynes & Parrotles  
his atty

# UNITED STATES PATENT OFFICE.

ADDISON H. BEALE, OF VANDERGRIFT, PENNSYLVANIA, ASSIGNOR TO AMERICAN SHEET & TIN PLATE COMPANY, OF PITTSBURG, PENNSYLVANIA, A CORPORATION OF NEW JERSEY.

## METHOD OF ROLLING METAL SHEETS.

No. 926,233.

Specification of Letters Patent.

Patented June 29, 1909.

Application filed May 11, 1908. Serial No. 432,077.

*To all whom it may concern:*

Be it known that I, ADDISON H. BEALE, of Vandergrift, in the county of Westmoreland and State of Pennsylvania, have invented a new and useful Method of Rolling Metal Sheets, of which the following is a full, clear, and exact description, reference being had to the accompanying drawings, forming part of this specification, in which—

10 Figure 1 is a sectional elevation, showing the first pack formed according to a preferred form of my method; and Fig. 2 is the second pack formed after rolling, opening, reforming the pack and doubling.

15 My invention relates to the rolling of sheets from metals which are difficult or impossible to roll to thin gages in the ordinary manner of sheet rolling. For example, in attempting to roll thin sheets from "Monel" 20 metal, it has been found that the metal breaks and will not draw out in rolling it into these thinner gages by itself. This Monel metal is an alloy of nickel and copper, with nickel predominating, and usually 25 in the proportion of about seventy-five per cent. of nickel to twenty-five per cent. of copper. It has certain desirable characteristics, especially as regards corrosion and hence sheets formed from it would have 30 commercial advantages. I have discovered that by sandwiching the plates or sheets of this Monel metal with soft plates of iron or steel, I can roll this Monel metal into thin gages successfully.

35 In carrying out the method in its preferred form, I roll out two sheet bars of soft steel and two sheet bars of Monel metal, as singles. I then make a pile of three of these rolled bars, as in Fig. 1, the outside bars 2, 2, being steel and the inner bar 3 being of Monel metal. This pile of three 40 is then reheated and rolled out, preferably to sufficient length to permit doubling. I then preferably open the pack and re-form 45 it, preferably by laying the plate or sheet of Monel metal on one or more of the steel sheets, and doubling this pack with the Monel metal on the inside. This re-formed pack, therefore, as shown in Fig. 2, consists 50 of a doubled Monel metal sheet 3<sup>a</sup>, with preferably two plies of steel 2<sup>a</sup> on each side thereof. Such pack is then reheated and rolled out to give the desired gage.

55 The advantages of my invention will be apparent to those skilled in the art, since a

practical and successful method is obtained for rolling sheets from alloys or metals which can not be rolled to thin gages by themselves. The steel appears to act both as a cushion for the other metal and also to aid in holding the heat in the other metal, when sandwiched, as above described.

My process is not to be confused with processes of rolling compound sheets, since the invention is designed to give sheets of a single metal or alloy, the final pack being opened after each pass to prevent these sheets from welding.

Many variations may be made in the process, for example, the piles may be varied as to the number of plies, the thickness of the bars or sheets may be varied, and the particular arrangement of the sheets may be changed without departing from my invention, which consists broadly in associating the bars or plates of the other metal or other alloy with bars or plates of soft iron or steel during the rolling operation.

I claim:

1. The method of producing thin sheets of metals or alloys of bad rolling qualities on account of breaking, &c., as compared with iron or steel, consisting in associating a bar or plate of said metal or alloy with a bar or plate of iron or steel, and then rolling and thereby elongating and thinning the same; substantially as described.

2. The method of producing thin sheets of metals or alloys of bad rolling qualities on account of breaking, &c., as compared with iron or steel, consisting in associating a bar or plate of said metal or alloy with a bar or plate of iron or steel, doubling the pack, and rolling and thereby elongating and thinning the doubled pack; substantially as described.

3. The method of producing thin sheets of metals or alloys of bad rolling qualities on account of breaking, &c., as compared with iron or steel, consisting in associating a bar or plate of said metal or alloy with a bar or plate of iron or steel, doubling the pack into a pack with the iron or steel forming the outer layers thereof, and then rolling and thereby elongating and thinning the doubled pack; substantially as described.

4. The method of producing thin sheets of metals or alloys of bad rolling qualities on account of breaking, &c., as compared with iron or steel, consisting in associating

a bar or plate of said metal or alloy with a bar or plate of iron or steel, doubling the pack with the iron or steel outside, reheating the pack, and rolling and thereby 5 elongating and thinning said doubled pack; substantially as described.

5. The method of producing thin sheets 10 of metals or alloys of bad rolling qualities on account of breaking, &c., as compared with iron or steel, consisting in sandwiching said metal or alloy between iron or steel sheets or plates, and rolling and thereby elongating and thinning the same; substantially as described.

15 6. The method of producing thin sheets

of metals or alloys of bad rolling qualities on account of breaking, &c., as compared with iron or steel, consisting in sandwiching the other metal or alloy between iron or steel sheets or plates, doubling the same with 20 the iron or steel outside, and then reheating and rolling and thereby elongating and thinning the same; substantially as described.

In testimony whereof, I have hereunto 25 set my hand.

ADDISON H. BEALE.

Witnesses:

R. G. SCOTT, Jr.,  
I. K. DARBAKER.